

July 9, 1940.

P. KEMP

2,207,461

SEPARATION OF THE CONSTITUENTS OF ALLOYS OR MIXTURES OF  
METALS AND/OR ELEMENTS SIMILAR TO METALS  
Filed Oct. 12, 1938



Inventor:

Paul Kemp,

Barley & Sharpen  
Attorneys

## UNITED STATES PATENT OFFICE

2,207,461

SEPARATION OF THE CONSTITUENTS OF  
ALLOYS OR MIXTURES OF METALS  
AND/OR ELEMENTS SIMILAR TO METALS

Paul Kemp, Vienna, Germany

Application October 12, 1938, Serial No. 234,631  
In Germany October 25, 1937

6 Claims. (Cl. 75—63)

This invention relates to an improvement of the known process for the decomposition of alloys and/or mixtures of metals and/or metal-like elements, by liquation.

5. An object of the invention is in particular to attain a particularly far-reaching separation of the more easily fusible parts of the alloy or of the mixture from the parts remaining solid in the liquation. 5

10. A further object of the invention is an especially effective aid to the separation of the constituents of the liquation product by the use of particularly suitable temperatures in the liquating process. 10

15. A further object of the invention is the carrying out of the liquation fractionally and separation of the liquation products at different temperatures. A further object of the invention is to facilitate the separating of certain constituents present in a small quantity as compared with the other constituents, of the initial material, during the liquation process itself. 15

In the decomposition of alloys or mixtures of metals and metal-like elements into constituents melting at different temperatures, by means of liquation, a sufficiently thorough separation of the liquid from the solid liquation products presents considerable difficulties. 20

All the known liquation processes have the common drawback that the separation of the liquation products is only very incomplete, since considerable quantities of the liquid portion are retained by the solid parts remaining in such manner that with alloys having only a small proportion of easily fusible constituents, these could not hitherto be separated successfully by liquation from the constituents melting at a higher temperature. This is true both for the usual process in which the alloy is heated on an inclined furnace sole and the components thus liquefied, flow off automatically in consequence of the inclination of the sole plate, and also in the other known processes in which the carrying out of the liquation takes place by complete melting of the alloys in a shaft made of masonry, slow cooling thereof to liquation temperature, and the draining off of the portion left liquid through a tapping hole. It is also true for the known processes in which the liquid parts are filtered off from the solid constituents through a base permeable to the liquid, if necessary using a certain pressure for accelerating the passage of the liquid, e. g., by evacuating the receiver. 30

35. I have found that an astonishingly far-reach-

ing removal of the liquid from the solid liquation constituents and thus a practically complete separation thereof from each other even with the presence of certain constituents only in very small quantities can be attained by pressing the liquated mixture of the solid and liquid constituents against a base permeable to the latter made, for example, of porous material, or against a grating provided with interruptions, e. g. holes or slots of suitable width, under a high pressure of not less than 100 atms. pressure for example of at least 500 atms. and preferably at least 1000 atms. The pressure can be produced either by compressed gas, or by mechanical means, e. g. by letting the pressure of a press piston act on the mixture of solid and liquid constituents at the liquation temperature, the mixture being placed in a press cylinder on a base permeable to the liquid parts. The pressures necessary according to the invention and also the desired working temperatures can be attained for example by the known hydraulic presses such as are used for making lead or brass tubes. 20

The "base" mentioned here and in the claims is not to be understood in the sense that this "base" must be underneath the liquated metal. It can be at the side or above the metal, so that the latter for example is forced in a piston press from below upward against a sieve plate closing the press cylinder at the top. 25

In carrying out the invention, the procedure may, for example, be adopted that the alloy or the metal mixture to be treated is heated up to liquation temperature in the press used for the liquation and is then subjected to a mechanical or gaseous pressure or, conversely, by the alloy or the mixture being placed in the liquid form in the press and after the cooling taking place therein to liquation temperature, being subjected to the pressure effect. In the first case, for example, when using a hydraulic press, the alloy or the mixture can be made into blocks adapted to the dimensions of the press cylinder, by pouring into chill moulds, the blocks being then heated in the press to the liquation temperature. 30

35. It has been found that it is possible according to the invention, to attain by the use of high pressures, a practically complete separation of the liquid from the solid liquation constituents and to thus permit with great completeness the decomposition of alloys or mixtures which contain only very little of the part fusing at a lower temperature. 40

45. The process according to the present invention is capable of very extended application. It 50

5

10

15

20

30

35

40

45

50

55

presents advantages in particular in cases in which eutectic mixtures are to be separated from impure alloys of the most varied kind, either on account of their actual value or to increase, by their separation, the value or the utility for certain purposes of the remaining alloy. As examples there may be mentioned: The production of mixed tin on the one hand, and white metal containing little lead, that is, speculum 10 metal on the other hand, from tin alloys of the most varied kind containing lead and copper. Furthermore, the removal of lead from bearing metal alloys containing much tin, the removal of tin and lead from impure zinc alloys, the 15 decomposition of hard lead alloys such as antimony-lead alloys with or without other metals into, on the one hand, the eutectic suitable as writing metal and, on the other hand, a press residue containing much antimony, as also the 20 removal of tin and antimony from old lead.

According to one method of carrying out the invention, there can be added to the alloy or to the metal mixture to be treated, and for the purpose of removing an injurious constituent, a 25 metal which combines with the injurious constituent and/or other constituents of the alloy or of the metal mixture in such a way that the separation desired is made possible. Thus, for example, in many cases, by the addition of a 30 metal which combines with the constituent to be removed, forming a compound melting at a higher temperature than the other constituents of the alloy, a separation of the troublesome constituent in the solid form is made possible 35 in the liquation. There may be mentioned as examples the removal of silver from lead by the addition of zinc and the removal of antimony from lead or tin alloys by the addition of aluminium. In consequence of the particularly 40 thorough separation of the liquid from the solid liquation products attainable by the high pressure to be used according to the invention, particularly favourable results can also be attained with this method of carrying out the invention.

45 In certain cases in particular when the quantity of the constituents contained in the initial alloy and to be separated out in solid form on the liquation, is only small, it is advisable to carry out a combined treatment in such manner that so as not to have to subject the whole alloy to the treatment with a high pressure, the main quantity of the liquid portion is first separated in known manner, e. g. by letting this run off on inclined furnace soles or by centrifuging, 50 or by filtering off under slight pressure, and then only the remaining liquation residue containing the solid constituents in a correspondingly increased concentration, is exposed to the action of high pressure, e. g. by means of a compressed gas 55 inert with respect to the alloy or by a press plunger. As in such cases in general the residue from the previous treatment is conveyed at once into the press or other device serving for the subsequent treatment under high pressure, the 60 necessity of heating or cooling is dispensed with, since the treatment under high pressure takes place at the same temperature as that of the preliminary treatment.

70 Special effects can also be attained in certain cases by a repeated pressing at different temperatures, whereby a fractional separation of an alloy or a metal mixture into a number of constituents is made possible. In this, the procedure may, for example, be adopted of either obtaining in the first place by liquation and pressing

at higher temperature a desired substance as press residue and the proportion pressed out in liquid form being again split up by reduction of temperature and renewed pressing, or by the alloy being at first only heated to such an extent that there take place a separation into a desired liquid constituent and a solid mixture, and after the separation of the latter by pressing this is split up by heating to a higher temperature with further renewed pressing out. 10

In the treatment of alloys or mixtures, the components of which have melting points differing greatly from each other, it is frequently of advantage to carry out the pressing treatment in the sense of the invention just below the melting point of the component melting at the higher temperature. 15

#### Examples

20 The treatment of the alloy takes place by means of the hydraulic press shown in longitudinal section in the drawing. In this 1 is the receptacle of the press cylinder, 4 the press piston, 2 is a sieve-like perforated matrix to be placed on the upper opening of the receptacle and which, together with the receiver vessel 5 for the expressed fluid metal can, by tightening the screw 3 in the manner shown by the drawing, be tightened on to the upper opening of the receptacle. 25 30 6 is a heating device, e. g. a gas burner.

The alloy to be treated is melted for example in an iron vessel and poured in portions each of about 20 to 30 kgs. into the receptacle 1 of the press cylinder previously heated for example by means of the burner 6. The matrix 2 with the receiver 5 is then placed in position and by tightening the screw 3, is closed tightly on to the upper opening of the receptacle. As soon as the alloy in the receptacle has cooled to the desired liquation temperature, in which the cooling process can if necessary be prolonged by means of the heating device 6, the press piston is placed under pressure and the pressure is raised in the course of about two minutes to approximately 1500 atms. The liquid expressed liquation portion passes through the perforations of the matrix into the container 5 where it then solidifies. After completion of the pressing-out process, the press plunger is relieved of pressure, the matrix after loosening the screw 3 is raised together with the container 5 and the pressed cake remaining in the receptacle is forced out by means of the press piston. The next portion of alloy can then at once be poured in and be treated in the same way as the first lot. In this manner for example 200 kgs. of metal can be easily dealt with per hour on a press operated by a single workman. 45

Naturally also, the procedure may be adopted of first letting the alloy placed in the fluid state in the receptacle 1 solidify completely, then heating this up to liquation temperature in the press cylinder by means of the heating device 6. If necessary, the alloy can also be placed in the receptacle of the press cylinder in lumps or in the form of a block adapted by casting in a separate mould, to the diameter of the receptacle, and this being then heated in the receptacle to liquation temperature. 50

75 By comparison, there were carried out tests with the same device and the same alloys, in which the liquid proportion of the liquated alloy was only driven through the whole of the matrix 2 at a pressure of 10 to 20 atms. 75

*Result of tests*

(1) From a tin alloy of 52% Sn, 21% Sb, 11% Cu, 16% Pb there are obtained in the above described manner at a temperature of between 180 5 and 190° C.:

(a) Using a pressure of 1500 atms.:

Liquid portion: 35% of mixed tin with 54.5% 10 of Sn, 3.5% of Sb, 0.2% of Cu, 41.8% of Pb.

Press residue: 65% of speculum metal with 50.5% of Sn, 30.4% of Sb, 16.9% of Cu, 2.0% of Pb. 15

(b) Using pressures of 10 to 20 atms.:

Liquid portion: 25% of mixed tin of the above 20 composition.

Press residue: 75% of speculum metal with 51.2% of Sn, 26.89% of Sb, 14.6% of Cu and 7.4% of Pb. 25

When using the lower pressure, not only has the yield in mixed tin been considerably reduced but also the composition of the speculum metal obtained as press residue has been so 25 altered that the metal has become practically valueless. For this metal is only suitable with a low content in lead, for making white metal bearings.

(2) From a hard lead alloy of 3.7% of Sn, 30 36.3% of Sb, 60% of Pb, there are recovered in the above-described manner at a temperature of between 240 and 255° C.:

(a) Using a pressure of 1500 atms.:

Liquid portion: 63% of eutectic with 3% of Sn, 35 13% of Sb, 84% of Pb, 37% of press residue consisting of 5% of Sn, 76% of Sb, 19% of Pb.

(b) Using pressure of 10 to 20 atms.:

Liquid portion: 45% of eutectic of the above 45 composition, 55% of press residue consisting of 4.3% of 4.3% of Sn, 55.3% of Sb and 40.4% of Pb.

As a high concentration in antimony is of outstanding importance for the utility of the press residue for alloy purposes and the press residue obtained with a pressure of only 10 to 20 atms. 50 has an antimony content which is too low for this purpose, by the use according to *a* of the

higher pressure a considerable more value press residue has been obtained.

What I claim is:

1. In the process of separating the constituents of metal mixtures and/or metal alloys by pressure liquation, the step comprising the separation of the liquid from the solid constituents by press extraction under a pressure of at least 500 atmospheres. 5

2. In the process of claim 1, which further comprises consecutively liquefying the various constituents and press extracting each liquid constituent under a pressure equal to at least 500 atmospheres. 10

3. In the process of claim 1 in which said metal mixture is composed of a tin alloy containing lead, the step of heating said metal mixture to obtain a liquid constituent composed of tin and a solid constituent composed of a tin alloy substantially free of lead, and press extracting 15 20 said liquid constituent under a pressure of at least 500 atmospheres.

4. In the process of claim 1 in which said metal mixture is composed of a tin alloy containing lead, the step of heating said metal mixture 25 at a temperature from approximately 180° C. to 190° C. to obtain a liquid constituent composed of tin and a solid constituent composed of a tin alloy substantially free of lead, and press extracting said liquid constituent under a pressure 30 of at least 500 atmospheres.

5. In the process for separating from an antimony-lead alloy an approximately eutectic lead and antimony alloys from lead alloys containing a substantially greater quantity of antimony and 35 having a higher melting point comprising heating said antimony-lead alloy to a temperature of approximately 240° C. to 255° C. to form a liquid eutectic constituent containing Sn, Sb, and Pb and a solid constituent containing lead and a large quantity of antimony, and press extracting 40 said liquid constituent under a pressure of at least 500 atmospheres.

6. In the process of separating from antimony alloyed with lead and tin a lead-tin alloy 45 and zinc substantially free of lead comprising heating said antimony-tin-lead alloy to a temperature of approximately 200° C. to 400° C. to form a solid constituent composed of zinc and a liquid constituent composed of lead and tin, and press extracting said liquid constituent under 50 a pressure of at least 500 atmospheres.

PAUL KEMP.